

## UNITED STATES PATENT OFFICE

2,603,562

NITROGEN CONTAINING STEELS WITH  
HIGH CREEP RESISTANCE AND HIGH  
TENSILE STRENGTH AT ELEVATED  
TEMPERATURESFranz Rapatz, Kapfenberg, Austria, assignor to  
Gebr. Böhler & Co. Aktiengesellschaft, Vienna,  
AustriaNo Drawing. Application February 27, 1948, Se-  
rial No. 11,857. In Germany November 27,  
1943Section 1, Public Law 690, August 8, 1946  
Patent expires November 27, 1963

2 Claims. (Cl. 75—123)

1

The present invention relates to steels with high creep resistance and high tensile strength at elevated temperatures containing nitrogen not combined with iron, chromium or manganese, but with metals which form nitrides of low solubility in steel such as elements of the 3rd group of the periodic system such as aluminium, the 4th group such as titanium and zirconium or the 5th group such as columbium. The effect of nitrogen already existing is increased to a surprising degree by the formation of stable nitrides of low solubility.

This increased effect is indicated by the following experimental results:

## Composition of the steels

|        | C per cent | Mn per cent | Total N per cent | Ti per cent | Zr per cent | N combined with Ti | N combined with Zr | Creep resistance 500° f by DVH method |
|--------|------------|-------------|------------------|-------------|-------------|--------------------|--------------------|---------------------------------------|
| 1..... | 0.10       | 0.3         | 0.20             |             |             |                    |                    | kg./mm. <sup>2</sup>                  |
| 2..... | 0.10       | 0.7         | 0.07             | 0.03        |             | 0.01               |                    | 4                                     |
| 3..... | 0.10       | 0.7         | 0.08             | 0.03        | 0.03        |                    | 0.0045             | 26                                    |

Similar values are also obtained when only elements of the 2nd group e. g. titanium- or zirconium-combined nitrogen are present. It is therefore apparent that presence of nitrogen alone is not sufficient, but what matters is the manner in which it is combined. In the case of steels as quoted in 2 and 3, values of creep resistance are obtained as are otherwise only obtained with relatively high additions of alloying metals (see "Die Edelstähle" by Dr. Rapatz, published by Springer, Berlin, 3rd edition, 1942, p. 145). According to the present invention the amount of alloying elements is very low—an important factor in view of the scarcity of such raw materials. What other metals may be used is a matter of the experimental technique applied. The quantity of insoluble nitride formed in the steel must not exceed 0.03%.

The strengthening effect of nitrogen seems to depend also on its state of distribution the latter being already controlled by the conditions prevailing in the heat. This favorable degree of distribution is reached, for example, if the nitrogen is first introduced into the steel in the form of nitrides of iron or chromium, and then elements of the 3rd group of the periodic system such as aluminium, the 4th group such as titanium and

zirconium or the 5th group as columbium are subsequently added to the steel already containing the nitrogen. The exact time when precipitation of the nitrides of low solubility takes place cannot be ascertained. They are, however, effectively present in the final state in the desired form.

The strengthening effect of nitrogen occurs equally on using steels according to the present invention for welding purposes. As nitrogen is absorbed from the air during the melting of the rod the addition of nitrogen to the welding wire by alloying becomes superfluous. It is only necessary that the elements of the 3rd group of the

2

periodic system such as aluminium, the 4th group as titanium and zirconium or the 5th group such as columbium which form nitrides of low solubility are present in the core wire or in the coating of the welding rod. In order to increase the creep resistance or tensile strength at elevated temperatures or for obtaining other effects, steels may be used which usually are alloyed with chromium, manganese, molybdenum, tungsten or nickel.

The invention is similarly applicable to structural steels having high creep resistance and also to tool steels which require creep resistance or high tensile strength at elevated temperatures, for example high grade steels intended for work at elevated temperatures and high speed steels.

45 I claim:

1. A steel having a high tensile strength, wear resistance and creep resistance containing a small quantity, not exceeding .03%, of the steel of a nitride selected from the group consisting of 50 aluminum, titanium, zirconium and columbium homogeneously distributed throughout the steel, said steel being produced by first dissolving in the molten steel a nitride of at least one metal selected from the group consisting of iron and 55 chromium in amounts sufficient to leave at least

.07% nitrogen in the steel upon solidification thereof, then adding to said molten steel solution containing said metal nitride a metal selected from the group consisting of aluminum, titanium, zirconium and columbium to convert a portion of the nitrides therein to nitrides of insoluble form homogeneously distributed throughout the steel.

2. A welded steel product having its joints welded by a steel having the composition as defined in claim 1.

FRANZ RAPATZ.

REFERENCES CITED

The following references are of record in the file of this patent:

UNITED STATES PATENTS

| Number    | Name   | Date          |
|-----------|--------|---------------|
| 1,352,534 | Russel | Nov. 14, 1920 |
|           |        | 20            |

| Number      | Name          | Date          |
|-------------|---------------|---------------|
| 2,022,307   | Austin        | Nov. 26, 1935 |
| 2,040,189   | Strauss       | May 12, 1936  |
| 2,121,055   | Smith et al.  | June 21, 1938 |
| 5 2,121,056 | Smith et al.  | June 21, 1938 |
| 2,174,740   | Graham et al. | Oct. 3, 1939  |
| 2,229,140   | Smith et al.  | Jan. 21, 1941 |
| 2,370,289   | Chandler      | Feb. 27, 1945 |

FOREIGN PATENTS

| Number  | Country     | Date          |
|---------|-------------|---------------|
| 195,385 | Switzerland | Apr. 16, 1938 |

OTHER REFERENCES

Mining and Metallurgical Investigations, Co-Operative Bulletin 66, pages 19 and 20. Edited by Herty, Jr., et al. Published by the Mining and Metallurgical Boards, Pittsburgh, Pennsylvania.